

## UNITED STATES PATENT OFFICE

2,024,408

METHOD OF TANNING HECTOGRAPH  
COPYING PADS

William B. Whitmore, Chicago, Ill., assignor to  
Ditto, Incorporated, Chicago, Ill., a corporation  
of West Virginia

No Drawing. Application August 11, 1933,  
Serial No. 684,765

11 Claims. (Cl. 41—31.6)

This invention relates to an improved method of tanning or hardening hectograph copying pads, or like gelatinous masses.

Copying surfaces have long been treated with various tanning agents for the purpose of rendering the product tougher, more resistant to heat, more lasting in operation and less tacky. Some agents such as formaldehyde are recognized to be rapid in their action, but their use is attended with difficulty in that control is uncertain, the mass is likely to become too viscous, or have its melting point raised too far before application to a backing material can be completed, and thus become unfit for use, and the final product is then under the best conditions not thoroughly suitable.

The slowly acting agents such as chrome alum and dichromates are easier to control, but take a very considerable length of time to complete the reaction. The tanning operation may require several months to be fully completed. The manufacturer is therefore forced to choose between having his product under-tanned at the outset, over-tanned before it is worn out, or else waiting several months before selling his product. Generally a compromise is reached under which the mass is somewhat under-tanned in the beginning and becomes over-tanned before otherwise wearing out. An over-tanned hectograph pad is unfit for use, however.

It has now been discovered that a light-sensitive slow-acting tanning agent may be applied to the gelatin mass and the tanning action accelerated by the use of strong light, particularly light in the ultra violet range. Under the influence of such light the reaction may be completed in a very few minutes, and a stabilized product is thus immediately formed.

The advantages of the new process are great and consist not only in the production of the pads in a very short period of time with the resulting saving in inventory and stock, but the product itself is actually improved by the short treatment. This improvement is at least two-fold. It is possible under this process to prepare special orders for special localities, which was impracticable where the material had to be stored several months before use. Even more important, however, is the basic improvement in the character of the gelatin, which is considerably more flexible in operation and absorbs water with greater facility.

The reason for this improved characteristic of the product is not fully understood, but is believed to be due to the fact that under the

former processes the water present in the mass dried out to a very considerable extent before the tanning operation became complete. During the drying-out process the size of the gelatin cells likewise decreased so that when the tanning or hardening operation was finished, the size of the cells was permanently fixed at this decreased level. On the other hand, when the tanning operation is carried out rapidly the size of the cells is unchanged. The evaporation of water subsequently, therefore, simply results in the collapse of the large cell walls, and upon subsequent moistening water is readily absorbed and the cells go back to their original size. The thickness of the large cell walls will of course be less than that of the small ones, which will likewise increase the ability of the mass to take up water rapidly.

As an example of the invention, a hectograph copying mass is prepared, for example, from one part of gelatin, four parts of water, 10 parts of glycerine, and 0.005 part of ammonium dichromate. After the mass has been applied to the backing material it is submitted to strong light, preferably regulated artificial light such as is produced by a carbon arc. A mercury quartz lamp used at a distance of 1½ to 2 feet over a period of 5 to 15 minutes, depending on the thickness of the band, will substantially complete the tanning operation. The exact time may readily be controlled by those skilled in the art both from the feel of the material and by the disappearance of the green color which is formed at the beginning of the tanning operation.

In place of the ammonium dichromate other alkali dichromates such as potassium and sodium may be employed.

The invention is likewise usable with other copying masses, and also for gelatin masses used for sizing paper. A typical example of a mixture suitable for the latter purpose is 1 part glue, 4 parts water, 7 parts glycerine and 0.008 parts ammonium dichromate. This mixture is applied to the paper and then treated with strong light as previously described.

By copying pad as used herein is meant not only a short pad, but other copying surfaces regardless of proportion or form.

The foregoing detailed description has been given for clearness of understanding only, and no unnecessary limitations should be understood therefrom, but the appended claims should be construed as broadly as permissible, in view of the prior art.

What I claim as new and desire to secure by Letters Patent is:

- 5 1. The method of forming stabilized hectograph copying surfaces which comprises forming a gelatinous mass containing a gelatin substance, water and glycerine wherein the proportion of glycerine exceeds the proportions of gelatin substance and of water, adding a minute proportion of a light-sensitive tanning agent to said gelatin mass and subjecting the mixture to the action of concentrated ultra violet light for a period sufficient to substantially complete said tanning.
- 10 2. The method for forming stabilized hectograph copying surfaces which comprises forming a gelatinous mass containing a gelatin substance, water and glycerine wherein the proportion of glycerine exceeds the proportions of gelatin substance and of water, adding a minute proportion of a light-sensitive tanning agent to said gelatin mass and substantially completing the tanning reaction with the aid of light in a period less than one week.
- 15 3. The method of forming stabilized hectograph copying surfaces which comprises forming a gelatinous mass containing a gelatin substance, water and glycerine wherein the proportion of glycerine exceeds the proportions of gelatin substance and of water, adding a light-sensitive tanning agent to said gelatin mass in amount not greater than about  $\frac{1}{2}\%$  based on the gelatin and carrying out the tanning reaction substantially solely under the influence of light.
- 20 4. The method as set forth in claim 3 in which the light is strong in the ultra violet component.
- 25 5. The method of forming stabilized hectograph copying surfaces which comprises forming a gelatinous mass containing a gelatin substance, water and glycerine wherein the proportion of glycerine exceeds the proportions of gelatin substance and of water, incorporating a minute proportion of a dichromate tanning agent in said gelatin mass and subjecting the mixture to the action of concentrated light for a period sufficient to substantially complete said tanning.
- 30 6. The method as set forth in claim 5, in which said tanning reaction is carried out substantially solely under the influence of light.
- 35 7. The method as set forth in claim 5, in which the tanning reaction is carried out substantially solely under the influence of a light source strong in ultra violet light.
- 40 8. The method of forming a surface on paper which comprises applying to said paper an aqueous gelatin base mass containing a major proportion of glycerine and including a dichromate tanning agent in minute proportion not greater than about  $\frac{1}{2}\%$  based on the gelatin content of said mass, and accelerating the tanning reaction by the application of strong light for a period sufficient to substantially complete said reaction.
- 45 9. The method of preparing stabilized hectograph copying surfaces which comprises preparing an aqueous gelatin base mass containing a major proportion of glycerine, applying said mass to a sheet of backing material and tanning said gelatin base mass under the influence of a minute proportion of a tanning agent having a non-reversible tanning action upon said gelatin, said tanning reaction being carried to substantial completion without the evaporation of a substantial quantity of moisture from said gelatin mass.
- 50 10. A hectograph copying pad comprising a backing material impregnated with hardened gelatin base mass comprising gelatin, a softening agent and a minute proportion of a light-active hardening agent, said mass being stable to the action of moderate heat and under absorption and evaporation of water, and the cells of said gelatin mass being of substantially the same size and wall thickness as when originally applied thereto.
- 55 11. A hectograph copying pad comprising a backing material impregnated with a gelatin base mass including a minute proportion of a dichromate tanning agent not greater than about  $\frac{1}{2}\%$  based on the gelatin contained in said mass, said gelatin having the characteristics resulting from promptly subjecting said mass to the action of strong ultra violet light until the tanning reaction is substantially complete and being substantially stabilized with respect to further hardening over substantial periods of time under conditions of use.

WILLIAM B. WHITMORE.